

Patented June 15, 1954

2,681,295

# UNITED STATES PATENT OFFICE

2,681,295

## PROCESS FOR FLAMEPROOFING TEXTILES WITH POLYPHOSPHONITRILIC ESTER

Carl Hamalainen, New Orleans, La., assignor to  
the United States of America as represented  
by the Secretary of Agriculture

No Drawing. Application December 5, 1952,  
Serial No. 324,427

3 Claims. (Cl. 117—137)

(Granted under Title 35, U. S. Code (1952),  
sec. 266)

1

A non-exclusive, irrevocable, royalty-free license in the invention herein described, for all governmental purposes, throughout the world, with the power to grant sublicenses for such purposes, is hereby granted to the Government of the United States of America.

This invention relates to the flameproofing of textiles such as threads and fabrics. More particularly, the invention provides a process of coating the fibers of a textile with a flameproofing agent which will remain on the fibers throughout numerous launderings.

In general, the process of the present invention comprises, reacting mixed polyphosphonitrilic chlorides with a chloro or bromo polyhalo-propyl alcohol in the presence of pyridine, impregnating a textile with the mixed esters so produced, and curing the wet textile.

Suitable polyphosphonitrilic chlorides include the high polymers of polyphosphonitrilic chloride and mixtures of the trimers and tetramers with the higher polymers. The mixed polyphosphonitrilic chlorides can suitably be employed in the form of a solute dissolved in the solvent in which they were prepared, solvents such as tetrachloroethane being particularly suitable.

The reaction between the polyphosphonitrilic chlorides and the alcohol is preferably conducted under anhydrous conditions at a temperature of about from 0 to 30° C. in the presence of sufficient pyridine to neutralize the hydrochloric acid formed.

Suitable polyhalopropyl alcohols include polyhalo propanols containing at least two halogen atoms of the group consisting of bromine and chlorine. The 2,3-dihalo alcohols are preferred, especially 2,3-dibromopropanol.

Textiles can suitably be flameproofed by impregnating them with the esters dissolved in a liquid solvent to form a solution containing from about 5 to 15% non-volatile materials, or emulsified with water to form an aqueous emulsion of a similar concentration. The reaction mixture in which the esters were produced can suitably be used per se. The use of acetone solutions of the esters containing from about 5 to 15% non-volatile materials is preferred. The esters can suitably be isolated from the reaction mixture by conventional methods such as pouring the reaction mixture into a selective solvent miscible with pyridine and the like and immiscible with the esters. Suitable selective solvents include water soluble alcohols such as methyl, ethyl, propyl and the like alcohols.

The impregnation of the textile can suitably be conducted by conventional textile impregnation procedures using one or a plurality of impregnation steps.

2

The textiles wet with the solution of the esters can suitably be cured by conventional textile curing procedures at temperatures ranging from about room temperature to the decomposition temperature of the textile for times ranging from a few minutes to several days, using the lower temperatures with the longer times. Where the tensile strength of the flameproof textile is important, the use of the lower temperatures is preferred.

The flameproofing agent provided by this invention can suitably be employed in conjunction with other flameproofing agents to enhance laundry-resistance, char length, and the like properties of the flameproofing ingredient.

The following examples are illustrative of the invention. In each case, the term "parts" refers to the parts by weight. The degree of flameproofing imparted to the various textile fabrics was measured by cutting the treated fabrics into strips approximately one cm. in width, fastening the strip so that the strip extends at an angle of about 45°, 90°, 135° or 180° from the fastener, and igniting the far end. With no flameproofing agent, the fabrics used in the examples failed to pass the "0° flameproofing test," i. e., the flame would propagate itself down a vertical strip of the fabric lighted at the top. A complete flameproof fabric will pass the 180° test, i. e., a vertical strip of the fabric will not support combustion when lighted at the bottom.

### Example 1

A solution of about 1 part of mixed polyphosphonitrilic chlorides dissolved in 10 parts of pyridine was mixed with about 5 parts of 2,3-dibromopropyl alcohol and allowed to react at room temperature (approximately 27° C.) for about 24 hours.

A piece of 80 sq. cotton cloth was impregnated with the reaction mixture (to a wet pickup of approximately 100%) and heated for 30 minutes at 110° C. The so-treated cloth passed the 180° flame test but was somewhat tendered.

A piece of similar cloth, similarly impregnated with the same reaction mixture, then dried 4 hours at room temperature, passed the 180° flame test and was not tendered. This latter sample passed the 180° flame test after 30 minutes boiling in 0.5% alkaline soap solution. After boiling in 2% sodium hydroxide solution for six hours this sample still passed the 135° flame test.

### Example 2

Five parts of a 20% solution of mixed polyphosphonitrilic chlorides in tetrachloroethane was mixed with 5 parts of pyridine and 4.5 parts of 2,3-dibromopropyl alcohol and allowed to re-

act for about 24 hours at room temperature. The reaction mixture was poured into about 40 parts ethyl alcohol. About 2.6 parts of a rubbery ester precipitated and were isolated.

Samples of 80 sq. cotton cloth were padded with 5%, 10% and 15% solutions of the above ester in acetone. One set of samples, series A, was allowed to air-dry overnight. The second set, series B, was cured in an oven for 30 minutes at 110° C. All of the samples were washed 15 minutes in running hot tap water and then dried in the oven 30 minutes at 110° C. All of the samples were subjected to 30 minutes boil in 0.5% alkaline soap solution and to 6 hours refluxing in aqueous 2% NaOH. Each of the latter treatments was followed by 15 minutes hot tap water washing and oven drying for 30 minutes at 110° C. The following table summarizes the flame tests and analyses of the so-treated samples.

| Samp. Nbr. | Treating Solution | Cure                    | Initial Increase In Wt., percent | Wt. Increase After Wash, percent | Flame Tests   |               |                |
|------------|-------------------|-------------------------|----------------------------------|----------------------------------|---------------|---------------|----------------|
|            |                   |                         |                                  |                                  | After Wash    | After Laundry | After 2% NaOH  |
| 1A         | 5% in acetone     | Air dry—overnight       | 7.8                              | 4.6                              | 90° (.54% P)  | 45°           | 45° (.36% P)   |
| 1B         | do                | Oven dry—30 min. 110° C | 7.2                              | 7.0                              | 135° (.77% P) | 90°           | 90° (.54% P)   |
| 2A         | 10% in acetone    | Air dry—overnight       | 13.9                             | 10.2                             | 135° (1.08%)  | 90°           | 90° (.64% P)   |
| 2B         | do                | Oven dry—30 min. 110° C | 13.6                             | 12.6                             | 180° (1.25%)  | 180°          | 135° (.98% P)  |
| 3A         | 15% in acetone    | Air dry—overnight       | 20.0                             | 16.2                             | 180° (1.59%)  | 180°          | 135° (1.04% P) |
| 3B         | do                | Oven dry—30 min. 110° C | 19.3                             | 17.0                             | 180° (1.58%)  | 180°          | 135° (1.27% P) |

### Example 3

A solution of about 1 part of mixed polyphosphonitrilic chlorides dissolved in about 10 parts pyridine was reacted with about 5 parts 1,3-dichloropropyl alcohol at room temperature for a period of about 24 hours.

A piece of 80 sq. cloth was impregnated with the reaction mixture (to a wet pickup of approximately 100%) and heated in the oven for 30

minutes at 110° C. After washing and drying, the sample had increased in weight by about 17%. The samples passed the 135° flame test.

I claim:

- 5 1. A process comprising, reacting mixed polyphosphonitrilic chlorides with a polyhalopropanol containing at least two atoms of the group consisting of bromine and chlorine in the presence of pyridine, impregnating a textile with the esters so produced, and curing the wet textile.
- 10 2. The process of claim 1 in which the polyhalopropanol is 2,3-dibromopropyl alcohol, and the textile is a cotton fabric.
- 15 3. A process of flameproofing cotton textiles comprising, impregnating the textiles with the esters produced by reacting a polyhalopropanol containing at least two atoms of the group consisting of bromine and chlorine with a mixture of polyphosphonitrilic chlorides in the presence of pyridine.
- 20

### References Cited in the file of this patent

#### UNITED STATES PATENTS

| Number     | Name           | Date           |
|------------|----------------|----------------|
| Re. 19,265 | Midgley et al. | Aug. 7, 1934   |
| 2,192,921  | Lipkin         | Mar. 12, 1940  |
| 2,427,997  | White          | Sept. 23, 1947 |
| 2,574,515  | Walter et al.  | Nov. 13, 1951  |
| 2,574,516  | Walter et al.  | Nov. 13, 1951  |